



US005902840A

# United States Patent [19]

Singh et al.

[11] Patent Number: 5,902,840

[45] Date of Patent: May 11, 1999

[54] **MODIFIED POLYMERIC AROMATIC ISOCYANATES HAVING ALLOPHANATE LINKAGES**

[75] Inventors: **Rina Singh**, Westerville; **Laurence G. Dammann**, Powell, both of Ohio

[73] Assignee: **Ashland Inc.**, Columbus, Ohio

[21] Appl. No.: **08/740,342**

[22] Filed: **Nov. 7, 1996**

[51] Int. Cl.<sup>6</sup> ..... **B22C 1/22**

[52] U.S. Cl. ..... **523/142**; 523/143; 525/395; 525/399; 528/49; 528/59; 164/6; 164/47

[58] Field of Search ..... 523/142, 143; 525/395, 399; 528/49, 59; 164/6, 47

## [56] References Cited

### U.S. PATENT DOCUMENTS

|           |         |                  |         |
|-----------|---------|------------------|---------|
| 3,769,318 | 10/1973 | Windemuth et al. | 260/471 |
| 4,160,080 | 7/1979  | König et al.     | 528/59  |
| 4,177,342 | 12/1979 | Bock et al.      | 528/45  |
| 4,396,738 | 8/1983  | Powell et al.    | 524/228 |
| 4,507,408 | 3/1985  | Torbus et al.    | 523/143 |
| 4,738,991 | 4/1988  | Narayan          | 521/124 |

|           |        |                |         |
|-----------|--------|----------------|---------|
| 4,760,101 | 7/1988 | Fechter et al. | 523/143 |
| 5,283,311 | 2/1994 | Narayan et al. | 528/49  |
| 5,319,053 | 6/1994 | Slack et al.   | 528/48  |
| 5,440,003 | 8/1995 | Slack          | 528/48  |
| 5,447,968 | 9/1995 | Barnett et al. | 523/142 |

### FOREIGN PATENT DOCUMENTS

994890 6/1965 United Kingdom .

Primary Examiner—Rachel Gorr  
Attorney, Agent, or Firm—David L. Hedden

## [57] ABSTRACT

The invention relates to modified polymeric aromatic isocyanates having allophanate linkages prepared by (a) reacting a polymeric aromatic isocyanate with a monofunctional aliphatic alcohol to form an intermediate modified polymeric isocyanate; and (b) reacting the intermediate modified polymeric isocyanate at an elevated temperature in the presence of a divalent metal catalyst. The invention also relates to foundry binder systems which use these modified polyisocyanates. These modified polyisocyanates, along with a phenolic resole resin, are added to a foundry aggregate to form a foundry mix which is shaped and cured with a gaseous amine curing catalyst by the cold-box process.

12 Claims, 1 Drawing Sheet

FIGURE 1



# MODIFIED POLYMERIC AROMATIC ISOCYANATES HAVING ALLOPHANATE LINKAGES

## FIELD OF THE INVENTION

This invention relates to modified polymeric aromatic isocyanates having allophanate linkages prepared by (a) reacting a polymeric aromatic isocyanate with a monofunctional aliphatic alcohol; and (b) then reacting the intermediate of step (a) at an elevated temperature in the presence of a divalent metal catalyst. These modified polymeric aromatic isocyanates, along with a phenolic resole resin, are added to a foundry aggregate to form a foundry mix which is shaped and cured with an amine curing catalyst by the cold-box process.

## BACKGROUND OF THE INVENTION

Several patents disclose the preparation of modified diisocyanates which contain allophanate linkages. See for instance British Patent 994,890 which discloses the reaction of diisocyanates with glycols and triols to form urethane polyisocyanates which are further reacted in the presence of heat and a metal catalyst to provide allophanate polyisocyanates. U.S. Pat. No. 4,738,991 teaches that the reaction of a molar excess of monomeric diisocyanates with polyhydric alcohols, which include both aliphatic and aromatic compounds such as ethylene glycol, trimethylene glycol, 1,4-butanediol, bisphenol A, thereof, in presence of certain specified catalysts produces polyisocyanates characterized by allophanate linkages. U.S. Pat. No. 5,319,053, U.S. Pat. No. 5,319,054, U.S. Pat. No. 5,44,003 teach that modified liquid diphenyl diisocyanate containing allophanate linkages can be synthesized from an aliphatic alcohol and monomeric diphenylmethane diisocyanate in presence of a catalyst. None of these patents disclose modified polymeric aromatic isocyanates containing allophanate linkages.

One of the major processes used in the foundry industry for making metal parts is sand casting. In sand casting, disposable foundry shapes (usually characterized as molds and cores) are made by shaping and curing a foundry mix which is a mixture of sand and an organic or inorganic binder. The binder is used to strengthen the molds and cores.

Two of the major processes used in sand casting for making molds and cores are the no-bake process and the cold-box process. In the no-bake process, a liquid curing agent is mixed with an aggregate and shaped to produce a cured mold and/or core. In the cold-box process, a gaseous curing agent is passed through a compacted shaped mix to produce a cured mold and/or core. Polyurethane-forming binders, cured with a gaseous tertiary amine catalyst, are often used in the cold-box process to hold shaped foundry aggregate together as a mold or core. See for example U.S. Pat. No. 3,409,579. The polyurethane-forming binder system usually consists of a phenolic resin component and polyisocyanate component which are mixed with sand prior to compacting and curing to form a foundry mix. None of the patents, previously discussed, which relate to modified diisocyanates containing allophanate linkages, suggest the use of such modified diisocyanates in foundry applications

## SUMMARY OF THE INVENTION

This invention relates to modified polymeric aromatic isocyanates containing allophanate linkages prepared by:

1. reacting a monofunctional aliphatic alcohol with a molar excess of a polymeric aromatic isocyanate having an isocyanate functionality of at least 2.2;

2. further reacting the product of step 1 at an elevated temperature in the presence of a catalytically effective amount of a divalent metal catalyst.

The modified polymeric isocyanates prepared by the process are complex products. They contain various polymeric structures and are characterized by C13 NMR as containing urethane along with allophanate linkages.

This invention also relates to polyurethane-forming foundry binder systems curable with a catalytically effective amount of an amine curing catalyst comprising as separate components:

- (A) a phenolic resin component; and
- (B) a polisocyanate component containing a modified a modified polymeric isocyanate having allophanate linkages.

The foundry binder systems are particularly useful for making foundry mixes used in the cold-box and no-bake fabrication processes for making foundry shapes. Foundry mixes are prepared by mixing component A and B with an aggregate. The foundry mixes are preferably used to make molds and cores by the cold-box process which involves curing the molds and cores with a gaseous tertiary amine. The cured molds and cores are used to cast ferrous and non ferrous metal parts. The modified polymeric aromatic isocyanates react with phenolic resins in a non-aqueous medium in the presence of an gaseous tertiary amine curing catalyst. The isocyanate (NCO) content decreases by the reaction of the polyisocyanate with the aliphatic alcohol. The amount of decrease depends upon the amount of modification, but there is still sufficient isocyanate content in the modified polyisocyanate to cure with the phenolic resin component.

The use of the modified polyisocyanates results in the improved release properties from molds and increased moisture resistance. It is believed their use also results in an increase in bulk cure and improved binder strength.

## BRIEF DESCRIPTION OF THE DRAWING

FIG. 1 shows the pressure needed to release a core from a corebox as the number of coremaking cycles increase. FIG. 1 compares the pressures needed to release cores from a corebox where the binders are made from unmodified polyisocyanates (outside the scope of the invention) to the pressures needed where the cores are made with modified polymeric aromatic isocyanates (within the scope of the invention).

## DETAILED DESCRIPTION OF THE INVENTION INCLUDING THE BEST MODE

The invention relates to storage stable modified polymeric aromatic isocyanates containing reactive isocyanate groups and allophanate linkages. The modified polymeric aromatic isocyanates are synthesized by reacting excess polymeric aromatic isocyanate with an aliphatic fatty alcohol to provide a polyurethane having reactive isocyanate groups which is further treated with a catalyst at an elevated temperature to yield polymers containing reactive isocyanate groups and polyallophanate linkages. For purposes of describing this invention, "polyisocyanate" includes "diisocyanate", and "polyisocyanates suitable for modification" includes any polyisocyanate. The polyisocyanate component of the binder system contains at least one modified polyisocyanate, and has a functionality of two or more, preferably 2 to 5.

The modified polymeric aromatic isocyanates can be diluted with unmodified polyisocyanates including aliphatic,

cycloaliphatic, aromatic, hybrid polyisocyanates, quasi-prepolymers, and prepolymers as mentioned before such as those used to prepare the modified polyisocyanates. The unmodified polyisocyanates typically have an NCO content of 2 weight percent to 50 weight percent, preferably from 15 to 35 weight percent. The amount of the modified polyisocyanate in the polyisocyanate component typically is from 1 weight percent to 100 weight percent based upon the total weight of the polyisocyanate in the polyisocyanate component, preferably from 2 weight percent to 16 weight percent.

The modified polymeric aromatic isocyanates typically have an NCO content from 1 to 50 weight percent, preferably from 12 to 33 weight percent after modification. Particular polymeric aromatic isocyanates which are suitable for modification with alcohols are polyisocyanates having an average functionality of at least 2.2. Representative examples of polymeric aromatic isocyanates include triisocyanates such as 4,4',4"-triphenylmethane triisocyanate, and toluene 2,4,6-triisocyanate; and the tetraisocyanates such as 4,4'-dimethylidiphenylmethane-2,2',5,5'-tetraisocyanate. Especially useful due to their availability and properties are diisocyanate, 4,4'-diphenylmethane diisocyanate, and polymeric polyisocyanates such as polymethylene polyphenylene polyisocyanate having a functionality of at least 2.3.

Suitable alcohols which can be used to modify the aromatic isocyanates can be represented by the following structural formula:



where R is a linear or branched aliphatic group having 2 to 50 carbon atoms, preferably from 6 to 30 carbon atoms. R can include, along its chain, carbon-carbon double or triple bonds, an aromatic ring, or even other functional groups as long as they are not reactive with the isocyanate. The hydrogen atoms in R can in addition be partially or totally replaced with fluorine atoms.

Representative examples of such alcohols include mono alcohols such as n-hexyl alcohol, n-heptyl alcohol, n-octyl alcohol, n-nonyl alcohol, n-decyl alcohol, lauryl alcohol, myristyl alcohol, cetyl alcohol, stearyl alcohol, arachidyl alcohol, behenyl alcohol, isohexyl alcohol, 2-ethyl hexanol, 2-ethyl isohexanol, iso octyl alcohol, phenethyl alcohol, isononyl alcohol, isodecyl alcohol, isotridecyl alcohol, isooctyl alcohol, isostearyl alcohol, oleyl alcohol, and linoleyl alcohol. Perfluorinated alcohols such as 1H, 1H, 5H-octafluoro-1-pentanol, 1H, 1H-heptafluoro-1-butanol, 1H, 1H-perfluoro-1-octanol, 1H, 1H, 2H, 2H-dodecafluoro-1-heptanol, N-ethyl-N-2-hydroxyethylperfluorooctane sulfonamide, and the like are also suitable. Mixtures of these alcohols can also be used.

The mole ratio of alcohol to polyisocyanate used to form the modified polyisocyanate is from 0.5 to 100 mole %, preferably about 0.5 to 50 mole %.

The intermediate alcohol modification is carried out by mixing the polyisocyanate and alcohol at room temperature and optionally heating to temperatures of 60° C. to 120° C. Also, the alcohol modification can be carried out in-situ at the required concentration by addition of the monofunctional aliphatic alcohol in presence of a catalyst. The intermediate, polyurethane-isocyanate is then further heated to 90° C. or 120° C. in presence of a suitable catalyst to provide the modified polymeric aromatic isocyanate. The modified polymeric aromatic isocyanate forming catalysts are used in the order of 100 to 300 mg in 100 parts of a given polyaromatic isocyanate.

Suitable divalent metal catalysts include zinc acetylacetone, cobalt 2-ethylhexanoate, cobalt naphthenate, and lead linoresinate. The preferred catalyst is zinc octoate. A catalyst stopper, such as acidic materials, e.g., anhydrous hydrochloric acid, sulfuric acid, bis(2-ethylhexyl)hydrogen phosphate, benzoyl chloride, Lewis acids and the like in the ratio of two equivalents of the acid to each mole of the zinc octoate can be employed. Typically the reactions are conducted without solvents, but solvents which are generally inert to the isocyanate, for example toluene, tetrahydrofuran or halogenated aromatic solvents can be employed.

The reaction according to the invention is carried out a temperature within the range of 90° C. to 120° C. The temperature can be increased before or after the catalyst is added and the temperature can be increased after the addition of the alcohol. The progress of the reaction according to the invention can be followed by determining the isocyanate content of the reaction mixture and Fourier Transform Infrared Spectroscopy. The C13 NMR spectra of the modified polymeric isocyanate shows a polymer having unreacted isocyanate groups and allophanate linkages, and can be used to determine the percentage of unreacted isocyanate allophanate linkages in the modified polymeric isocyanate, as well as the purity of the modified polymeric isocyanate. Preferably, the ratio of unreacted NCO groups to allophanate linkages in the modified polymeric isocyanate is from 2 to 1, preferably from 7 to 1.

The phenolic resin component of the binder system comprises a phenolic resole resin, preferably a polybenzyllic ether phenolic resin. The phenolic resole resin is prepared by reacting an excess of aldehyde with a phenol in the presence of either an alkaline catalyst or a divalent metal catalyst according to methods well known in the art. Solvents, as specified, are also used in the phenolic resin component along with various optional ingredients such as adhesion promoters and release agents.

The polyisocyanates are used in sufficient concentrations to cause the curing of the polybenzyllic ether phenolic resin with an amine curing catalyst. In general the isocyanate ratio of the polyisocyanate to the hydroxyl of the polybenzyllic ether phenolic resin is from 0.75:1.25 to 1.25:0.75, preferably about 0.9:1.1 to 1.1:0.9. The polyisocyanate is used in a liquid form. Solid or viscous polyisocyanates must be used in the form of organic solvent solutions, the solvent generally being present in a range of up to 80 percent by weight of the solution.

The polybenzyllic ether phenolic resin is prepared by reacting an excess of aldehyde with a phenol in the presence of a divalent metal catalyst according to methods well known in the art. The polybenzyllic ether phenolic resins used to form the subject binder compositions are polybenzyllic ether phenolic resins which are specifically described in U.S. Pat. No. 3,485,797 which is hereby incorporated by reference into this disclosure.

These polybenzyllic ether phenolic resins are the reaction products of an aldehyde with a phenol. They preferably contain a preponderance of bridges joining the phenolic nuclei of the polymer which are ortho-ortho benzyllic ether bridges. They are prepared by reacting an aldehyde and a phenol in a mole ratio of aldehyde to phenol of at least 1:1, generally from 1.1:1.0 to 3.0:1.0 and preferably from 1.1:1.0 to 2.0:1.0, in the presence of a metal ion catalyst, preferably a divalent metal ion such as zinc, lead, manganese, copper, tin, magnesium, cobalt, calcium, or barium.

Generally, the phenols used to prepare the phenolic resole resins may be represented by the following structural formula:



where B is a hydrogen atom, or hydroxyl radicals, or hydrocarbon radicals or oxyhydrocarbon radicals, or halogen atoms, or combinations of these. Multiple ring phenols such as bisphenol A may be used.

Specific examples of suitable phenols used to prepare the polybenzyllic ether phenolic resins include phenol, o-cresol, p-cresol, p-butylphenol, p-amylphenol, p-octylphenol, and p-nonylphenol.

The aldehydes reacted with the phenol include any of the aldehydes heretofore used to prepare polybenzyllic ether phenolic resins such as formaldehyde, acetaldehyde, propionaldehyde, furfuraldehyde, and benzaldehyde. In general, the aldehydes employed have the formula R'CHO wherein R' is a hydrogen or a hydrocarbon radical of 1 to 8 carbon atoms. The most preferred aldehyde is formaldehyde.

The polybenzyllic ether phenolic resin is preferably non-aqueous. By "non-aqueous" is meant a polybenzyllic ether phenolic resin which contains water in amounts of no more than about 10%, preferably no more than about 1% based on the weight of the resin. The polybenzyllic ether phenolic resin used is preferably liquid or soluble in an organic solvent.

Solubility in an organic solvent is desirable to achieve uniform distribution of the phenolic resin component on the aggregate. Mixtures of polybenzyllic ether phenolic resins can be used.

Alkoxy-modified polybenzyllic ether phenolic resins may also be used as the phenolic resin. These polybenzyllic ether phenolic resins are prepared in essentially the same way as the unmodified polybenzyllic ether phenolic resins previously described except a lower alkyl alcohol, typically methanol, is reacted with the phenol and aldehyde or reacted with an unmodified phenolic resin.

In addition to the polybenzyllic ether phenolic resin, the phenolic resin component of the binder composition also contains at least one organic solvent. Preferably the amount of solvent is from 40 to 60 weight percent of total weight of the phenolic resin component. Specific solvents and solvent combinations will be discussed in conjunction with the solvents used in the polyisocyanate component.

Those skilled in the art will know how to select specific solvents for the phenolic resin component and polyisocyanate component. The organic solvents which are used with the polybenzyllic ether phenolic resin in the polybenzyllic ether phenolic resin component are aromatic solvents, esters, ethers, and alcohols, preferably mixtures of these solvents.

It is known that the difference in the polarity between the polyisocyanate and the polybenzyllic ether phenolic resins restricts the choice of solvents in which both components are compatible. Such compatibility is necessary to achieve complete reaction and curing of the binder compositions of the present invention. Polar solvents of either the protic or aprotic type are good solvents for the polybenzyllic ether phenolic resin, but have limited compatibility with the polyisocyanate.

The polar solvents should not be extremely polar such as to become incompatible with the aromatic solvent. Suitable

polar solvents are generally those which have been classified in the art as coupling solvents and include furfural, furfuryl alcohol, Cellosolve acetate, butyl Cellosolve, butyl Carbitol, diacetone alcohol, and Texanol. Other polar solvents include 5 liquid dialkyl esters such as dialkyl phthalate of the type disclosed in U.S. Pat. No. 3,905,934 and other dialkyl esters such as dimethyl glutarate.

Aromatic solvents, although compatible with the polyisocyanate, are less compatible with the phenolic resins. 10 It is, therefore, preferred to employ combinations of solvents and particularly combinations of aromatic and polar solvents. Suitable aromatic solvents are benzene, toluene, xylene, ethylbenzene, and mixtures thereof. Preferred aromatic solvents are mixed solvents that have an aromatic 15 content of at least 90% and a boiling point range of 138° C. to 232° C.

Limited amounts of aliphatic and/or cycloaliphatic solvents or mixtures thereof may be used with the polyisocyanate component. Examples of such solvents are mineral 20 spirits, kerosene, and naphthas. Minor amounts of aromatic solvent may also be present in the solvents.

It may also be useful to add a bench life extender to the binder. A bench life extender retards the premature reaction of the two components of the binder system after they are 25 mixed with sand. Premature reaction reduces flowability of the foundry mix and causes molds and cores made with the sand mix to have reduced strengths. The bench life extender is usually added to the polyisocyanate component of the binder. Examples of bench life extenders are organic 30 phosphorus-containing compounds such as those described in U.S. Pat. No. 4,436,881 and U.S. Pat. No. 4,683,252, and inorganic phosphorus-containing compounds such as those described in U.S. Pat. No. 4,540,724 and U.S. Pat. No. 4,602,069, all of which are hereby incorporated by reference. 35 The amount of bench life extender used in the polyisocyanate component is generally from 0.01 to 3.0 weight percent, preferably 0.1 to 0.8 weight percent based upon the total weight of the binder.

Drying oils, for example those disclosed in U.S. Pat. No. 40 4,268,425, may also be used in the polyisocyanate component. Drying oils may be synthetic or natural occurring and include glycerides of fatty acids which contain two or more double bonds whereby oxygen on exposure to air can be absorbed to give peroxides which catalyze the polymerization 45 of the unsaturated portions.

Other optional ingredients include release agents and a silane, which is used to improve humidity resistance. See for example, U.S. Pat. No. 4,540,724, which is hereby incorporated into this disclosure by reference.

50 The binder system is preferably made available as a two-package system with the phenolic resin component in one package and the polyisocyanate component in the other package. Usually, the binder components are combined and then mixed with sand or a similar aggregate to form the foundry mix or the mix can be formed by sequentially mixing the components with the aggregate. Preferably the phenolic resin component is first mixed with the sand before mixing the isocyanate component with the sand. Methods of distributing the binder on the aggregate particles are well-known to those skilled in the art. The mix can, optionally, 55 contain other ingredients such as iron oxide, ground flax fibers, wood cereals, pitch, refractory flours, and the like.

Various types of aggregate and amounts of binder are used to prepare foundry mixes by methods well known in the art. 60 Ordinary shapes, shapes for precision casting, and refractory shapes can be prepared by using the binder systems and proper aggregate. The amount of binder and the type of 65

aggregate used is known to those skilled in the art. The preferred aggregate employed for preparing foundry mixes is sand wherein at least about 70 weight percent, and preferably at least about 85 weight percent, of the sand is silica. Other suitable aggregate materials for ordinary foundry shapes include zircon, olivine, aluminosilicate, chromite sands, and the like.

In ordinary sand type foundry applications, the amount of binder is generally no greater than about 10% by weight and frequently within the range of about 0.5% to about 7% by weight based upon the weight of the aggregate. Most often, the binder content for ordinary sand foundry shapes ranges from about 0.6% to about 5%, preferably about 1% to about 5% by weight based upon the weight of the aggregate in ordinary sand-type foundry shapes.

Although the aggregate employed is preferably dry, small amounts of moisture, generally up to about 1.0 weight percent, more typically less than 0.5 weight percent, based on the weight of the sand, can be tolerated. This is particularly true if the solvent employed is non-water-miscible or if an excess of the polyisocyanate necessary for curing is employed since such excess polyisocyanate will react with the water.

The foundry mix is molded into the desired shape, whereupon it can be cured. Curing can be affected by passing a tertiary amine through the molded mix such as described in U.S. Pat. No. 3,409,579 which is hereby incorporated into this disclosure by reference.

The examples will illustrate specific embodiments of the invention. These examples along with the written description will enable one skilled in the art to practice the invention. It is contemplated that many other embodiments of the invention will be operable besides these specifically disclosed.

## EXAMPLES

Examples 1-4 illustrate the preparation of modified polyisocyanates within the scope of this invention. Examples 5-6 illustrate the use of the modified polyisocyanates in foundry binder systems to make foundry cores by the cold-box process with and without a release agent. The tensile strengths were determined on a Thwing Albert Intelect II—Std. Instrument Company, Philadelphia, USA 19154 tensile tester. In all of the examples the test specimens were produced by the cold-box process by contacting the compacted mixes with triethylamine (TEA) for 1.0 second. All parts are by weight and all temperatures are in °C. unless otherwise specified. The following abbreviations are used in the examples:

|              |   |                                                                                                                                                                                                                                                |
|--------------|---|------------------------------------------------------------------------------------------------------------------------------------------------------------------------------------------------------------------------------------------------|
| MONDUR MRS 5 | = | a polymethylene polyphenyl isocyanate sold by Bayer AG having a free NCO content of 32% and a functionality of 2.4.                                                                                                                            |
| MONDUR MR    | = | a polymethylene polyphenyl isocyanate sold by Bayer AG having a free NCO content of 32% and a functionality of 2.7.                                                                                                                            |
| MPAIA        | = | modified polymeric aromatic isocyanate having allophanate linkages                                                                                                                                                                             |
| RESIN        | = | a polybenzyl ether phenolic resin prepared with zinc acetate dihydrate as the catalyst and modified with the addition of 0.09 mole of methanol per mole of phenol prepared along the lines described in the examples of U.S. Patent 3,485,797. |

## EXAMPLE 1

To a three neck-round bottom flask, equipped with a condenser, mechanical stirrer and dropping funnel, under an atmosphere of nitrogen was added Mondur MRS-5 (100 grams, 32.35% NCO content) and to this was added oleyl alcohol (4 mol %, 9.6 mLs, 8 grams) dropwise at room temperature, over a period of ten minutes. The reaction was heated at 60° C. for 1 hour to provide an oleyl modified isocyanate having a 28% NCO content and a viscosity of 1.17 poise at room temperature (25° C.) determined by Carri-Med rheometer. To the reaction mixture at 60° C. was added 400 mg of a 22% zinc octoate catalyst (zinc hex-chem supplied by Mooney Chemicals, Inc.) and it was heated to 120° C. for 4 hrs. The reaction mixture was cooled to 90° C., and benzoyl chloride (800 mg) was added and further stirred for 30 minutes to ensure the reaction was terminated. Upon cooling to room temperature, a dark colored liquid was obtained as the modified polymeric aromatic isocyanate having allophanate linkages (MPAIA) having a viscosity of 3.70 poise (25° C.) and a 23.6% NCO content. The calculated allophanate group content of the product was 8.8%. Fourier Transform Infrared spectrum provides the bands characteristic of allophanate formation at 1725 cm<sup>-1</sup> and 1685 to 1690 cm<sup>-1</sup>, and does not provide any indication of secondary products with an isocyanurate structure. The C13 NMR spectrum showed signals at 156 ppm and 151.5 ppm in the carbonyl range (corresponding to allophanate structures) and 120 ppm (corresponding to isocyanate structures).

Optionally, the reaction was conducted with the catalyst (zinc octoate) added at the same time as the polyisocyanate (Mondur MRS-5) and alcohol (oleyl), and the reaction was heated at 120° C. for 4 hours. The percent NCO content and the calculated allophanate group content of the product were similar to that obtained when the reaction was conducted with the catalyst added after the formation of the polyurethane-isocyanate. The C13 NMR was run on a Varian 400 MHz NMR in deuteriated chloroform. Samples for Gel Permeation Chromatography (GPC) analyses were prepared by adding 0.10 gram of material to 10 mL of tetrahydrofuran (THF). The mixtures were allowed to stand for 24 hours to dissolve the polymer and then filtered through a 0.45 mm Acrodisc PTFE filter for injection into the GPC. The analyses of the samples by GPC were run on a Waters GPC600 at 40° C. using a Waters HR1/HR2 column set and using polystyrene as standards. The average molecular weight (Mw) and the average number molecular weight (Mn) of the polymers were: polyurethane-isocyanate: Mw=550, Mn=216 (Mw/Mn=2.55), MPAIA: Mw=792, Mn=265 (Mw/Mn=2.98). The polymers were storage stable under an atmosphere of nitrogen for weeks. Crystallization in either of the polymers was not observed.

## EXAMPLE 2

In accordance with the procedure set forth in Example 1, oleyl alcohol (20 grams) was added to Mondur MRS-5 (100 grams, 32.35% NCO content) which resulted in an isocyanate content of 24% of the polyurethane-isocyanate and a viscosity of 1.55 poise at room temperature (25° C.). The modified polymeric aromatic isocyanate having allophanate linkages (MPAIA) obtained had a viscosity of 3.82 poise at room temperature (25° C.) and a NCO content of 16.2%. The calculated allophanate group content of the MPAIA was 16.2%. The average weight (Mw) and the average number weight (Mn) of the polymers were: polyurethane-isocyanate: Mw=584, Mn=235 (Mw/Mn=2.48), MPAIA: Mw=999, Mn=327 (Mw/Mn=3.05).

## EXAMPLE 3

In accordance with the procedure set forth in example 1, oleyl alcohol (8 grams) was added to Mondur MR (100 grams, 31.75% NCO content) which resulted in an isocyanate content of 28% of the polyurethane-isocyanate and a viscosity of 3.58 poise at room temperature (25° C.). The MPAIA obtained had a viscosity of 4.89 poise at room temperature (25° C.) and a NCO content of 24.3%. The calculated allophanate group content of the product was 7.5%. The average weight (Mw) and the average number weight (Mn) of the polymers were: polyurethane-isocyanate: Mw=664, Mn=259 (Mw/Mn=2.56), MPAIA: Mw=902, Mn=321 (Mw/Mn=2.80).

## EXAMPLE 4

In accordance with the procedure set forth in example 1, oleyl alcohol (20 grams) was added to Mondur MR (100 grams, 31.75% NCO content) which resulted in an isocyanate content of 23% of the polyurethane-isocyanate and a viscosity of 12.08 poise at room temperature (25° C.). The MPAIA obtained had a viscosity of 15.62 poise at room temperature (25° C.) and a NCO content of 14.7%. The calculated allophanate group content of the product was 17.1%. The average weight (Mw) and the average number weight (Mn) of the polymers were: polyurethane-isocyanate: Mw=836, Mn=314 (Mw/Mn=2.66), MPAIA: Mw=1498, Mn=446 (Mw/Mn=3.36).

## COMPARISON A AND EXAMPLES 5-6

(Formulations without a Release Agent.)

Comparsion A and Examples 5-6 illustrate the preparation of a foundry test shape (dogbone shape). Comparison A uses an unmodified polyisocyanate while Example 5 and 6 use the modified polyisocyanate of Examples 4, or dilutions thereof, in a polyurethane-forming binder system containing no release agent. The formulations for Part I and Part II of the binder system are given in Table I.

TABLE I

| (FORMULATION OF BINDER)            |           |              |      |                                        |       |       |       |
|------------------------------------|-----------|--------------|------|----------------------------------------|-------|-------|-------|
| PART I (RESIN COMPONENT)           |           |              |      |                                        |       |       |       |
| COMPONENT                          |           | AMOUNT (pbw) |      |                                        |       |       |       |
| RESIN                              |           | 55.0         |      |                                        |       |       |       |
| ALIPHATIC SOLVENT                  |           | 14.0         |      |                                        |       |       |       |
| AROMATIC SOLVENTS                  |           | 23.3         |      |                                        |       |       |       |
| SILANE                             |           | 0.8          |      |                                        |       |       |       |
| PART II (POLYISOCYANATE COMPONENT) |           |              |      |                                        |       |       |       |
| MODIFIED POLYISOCYANATE (MPI)      |           |              |      | UNMODIFIED POLYISO-CYANATE (MONDUR MR) |       |       |       |
| Example                            | MPI       | pbw          | wt % | wt %                                   | oleyl | pbw   | wt. % |
| Comparsion A                       | None      | 0            | 0    | 0                                      |       | 73.3  | 100   |
| Example 5                          | Example 4 | 18.33        | 25   | 4.2                                    |       | 54.98 | 75    |
| Example 6                          | Example 4 | 36.65        | 50   | 8.4                                    |       | 36.65 | 50    |
| AROMATIC SOLVENTS                  |           |              |      | 23.6                                   |       |       |       |
| MINERAL SPIRITS                    |           |              |      | 2.3                                    |       |       |       |
| BENCH LIFE EXTENDER                |           |              |      | 0.8                                    |       |       |       |

In Examples A and 5-6, cores were made with the binders of Examples A and 5-6, as described in Table I, by mixing

## 10

sand with these formulations. The sand mix (Manley 1L5W lake sand) included 55 weight percent of Part I and 45 weight percent of Part II (Table I). The sand mixture contained 1.5 weight percent of binder in 4000 parts of 5 Manley 1L5W lake sand.

The resulting foundry mixes were compacted into a dogbone shaped core box by blowing and were cured using the cold-box process as described in U.S. Pat. No. 3,409, 10 579. In this instance, the compacted mixes were then contacted with a mixture of TEA in nitrogen at 20 psi for 1.0 second, followed by purging with nitrogen that was at 60 psi for about 6 seconds, thereby forming AFS tensile test specimens (dog bones) using the standard procedure. The 15 test shapes were obtained using a REDFORD CBT-1 core blower.

The tensile strengths of the dogbone shaped cores, made with a foundry mix having zero benchlife, were measured immediately (1 minute), 3 hours, 24 hours, and 24 hours 20 after being stored at 100% relative humidity at ambient conditions in closed containers. They were also measured immediately and 24 hours after gasssing with TEA after the foundry mix had a benchlife of three hours. Measuring the tensile strength of the dog bone shapes enables one to predict 25 how the mixture of sand and binder will work in actual foundry operations. Lower tensile strengths for the shapes indicate that the phenolic resin and polyisocyanate reacted more extensively after mixing with the sand prior to curing.

30 The tensile properties of the modified polymeric aromatic isocyanate having allophanate linkages (MPAIA) made from the binders of Examples 5-6, based on Mondur MR, are shown in Table II. Example B is the similar to Example A except it contains an internal release agent and is compared to Example A, 5 and 6 which do not contain an internal release.

TABLE II

| TENSILE STRENGTHS OF TEST CORES PREPARED WITH MODIFIED AND UNMODIFIED MONDUR MR WITHOUT AN INTERNAL RELEASE AGENT |     |     |     |     |  |
|-------------------------------------------------------------------------------------------------------------------|-----|-----|-----|-----|--|
| TENSILE STRENGTHS (psi)                                                                                           |     |     |     |     |  |
| EXAMPLE                                                                                                           | A   | B   | 5   | 6   |  |
| ZERO BENCH (1 MIN)                                                                                                | 162 | 142 | 145 | 105 |  |
| ZERO BENCH (1 HR)                                                                                                 | 220 | 199 | 189 | 152 |  |
| ZERO BENCH (24 HR)                                                                                                | 230 | 207 | 206 | 191 |  |
| HUMIDITY @ 100%                                                                                                   | 52  | 44  | 105 | 150 |  |
| 3 HR BENCH LIFE (IMMEDIATE)                                                                                       | 124 | 118 | 143 | 101 |  |
| 3 HR BENCH LIFE (24 HR)                                                                                           | 189 | 178 | 191 | 143 |  |

50 Table II indicates that the humidity resistance of the cores increased when modified polyisocyanates were used without a corewash. The data further indicate that the humidity resistance increases even more as the amount of modification to the polyisocyanate by the oleyl alcohol is increased.

## EXAMPLES 7-8

60 (Determining Release Properties Where No Release Agent was Used in Binder System.)

Using a cylinder sticking test, release properties were determined for cores made with binders containing a conventional unmodified polyisocyanate (comparison binder system with MONDUR MR), and the binders of Example 5 (4.2 weight percent of oleyl alcohol) and Example 6 (8.4

## 11

weight percent of oleyl alcohol), (see Table I) containing the MPIA. None of the binder systems contained the internal release agent.

The cylinder sticking test, used to test the release properties of cores made with the binder systems, involved repeatedly blowing Manley 1L5W Lake sand into a 2x4 inch stainless steel cylinder where it was cured with TEA. A tensile tester was used to determine the pressure (lbs) it would take to remove the cured cylindrical sand from the steel cylinder.

The binder level was 1.5 weight percent with 55 weight percent of Part I and 45 weight percent of Part II in the formulation.

The core blower used was a Redford CBT-1 with a gassing pressure of 20 psi, and blow pressure of 60 psi. The tensile tester to measure the pressure was a QC-1000 Tensile Tester Thwing-Albert Instrument Company, Philadelphia, USA 19154.

Table IV, the results of which are graphically depicted in FIG. 1, shows data which results from comparing a commercial polyisocyanate, MONDUR MR with polyisocyanate components which contain polyisocyanates prepared with 4.2 (Example 5) and 8.4 (Example 6) weight percent oleyl alcohol. The formulations for the binders are shown in Table 1. FIG. 1 shows the pressures of the oleyl modified polyisocyanates being much lower than the unmodified polyisocyanates, i.e., the modified polyisocyanates have a much better release property. Also, with increasing levels of the oleyl alcohol in the polyisocyanate backbone gives pressures which are even lower than the unmodified polyisocyanates. The oleyl alcohol modified polyisocyanates gave excellent release properties in comparison to the unmodified polyisocyanates. Similar results are shown when the modified polyisocyanates are compared to MONDUR MRS-5.

TABLE IV

## COMPARISON OF CORE RELEASE FOR BINDERS MADE WITH UNMODIFIED POLYISOCYANATES AND MODIFIED POLYISOCYANATES

| EXAMPLE      | CYCLES |     |     |     |     |     |     |     |     |     |
|--------------|--------|-----|-----|-----|-----|-----|-----|-----|-----|-----|
|              | 1      | 5   | 10  | 15  | 20  | 25  | 30  | 40  | 50  | 60  |
| Comparison C | 78     | 167 | 267 | 276 | 290 | 307 |     |     |     |     |
| 7            | 97     | 47  | 55  | 94  | 118 | 120 | 119 | 130 | 126 | 130 |
| 8            | 9      | 17  | 23  | 27  | 26  | 42  | 56  | 54  | 64  | 72  |

We claim:

1. A foundry mix comprising:
  - (A) a major amount of aggregate; and
  - (B) an effective bonding amount of a polyurethane-forming binder system curable with a catalytically effective amount of an amine curing catalyst comprising as separate components:
    - (1) a phenolic resin component; and
    - (2) a polyisocyanate component comprising a modified polymeric aromatic isocyanate having allophanate linkages prepared by:
      - (a) reacting a monofunctional aliphatic alcohol with a molar excess of an aromatic polyisocyanate having an isocyanate functionality of at least 2.2;
      - (b) further reacting the product of step (a) at an elevated temperature in the presence of a catalytically affective amount of a divalent metal catalyst.

50

ment is from 2 weight percent to 16 weight percent, where said weight percent is based upon the total weight of the polyisocyanate in the polyisocyanate component.

12. A process for preparing a foundry shape which comprises:

- (a) forming a foundry mix as set forth in any of claims 1, 2, 3, 4, 5, 6, 7, 8, 9, 10, and 11;
- (b) forming a foundry shape by introducing the foundry mix obtained from step (a) into a pattern;
- (c) contacting the shaped foundry mix with a tertiary amine catalyst; and
- (d) removing the foundry shape of step (c) from the pattern.

55

60

## 12

2. The foundry mix of claim 1 wherein the binder composition is about 0.6 to 5.0 weight percent based upon the weight of the aggregate.

3. The foundry mix of claim 2 wherein the modified polymeric aromatic isocyanate has an NCO content of from 12 to 33 weight percent after modification.

4. The foundry mix of claim 3 wherein the polyisocyanate component also contains an unmodified polyisocyanate and the mole ratio of unmodified polyisocyanate to modified polymeric aromatic polyisocyanate is from 20:1 to 1:1.

10 5. The foundry mix of claim 4 wherein the aromatic isocyanate used to prepare the modified polymeric polyisocyanate is selected from the group consisting of 4,4'-diphenylmethane diisocyanate, and polymethylene polyphenylene polyisocyanate.

15 6. The foundry mix of claim 5 wherein the monofunctional alcohol is selected from the group consisting of isocetyl alcohol, isostearyl alcohol, oleyl alcohol, and mixtures thereof.

20 7. The foundry mix of claim 6 wherein the phenolic resin component comprises a (a) a polybenylic ether phenolic resin prepared by reacting an aldehyde with a phenol such that the molar ratio of aldehyde to phenol is from 1.1:1 to 3:1 in the presence of a divalent metal catalyst, and (b) a solvent in which the resole resin is soluble.

25 8. The foundry mix of claim 7 wherein the ratio of hydroxyl groups of the polybenylic ether phenolic resin to the isocyanate groups of the polyisocyanate hardener is from 0.80:1.2 to 1.2:0.80.

30 9. The foundry mix of claim 8 wherein the ratio of unreacted NCO groups to allophanate linkages in the modified polymeric isocyanate is from 2:1 to 7:1.

10. The foundry mix of claim 9 where the monofunctional alcohol is oleyl alcohol.

11. The foundry mix of claim 10 wherein the amount of the modified polyisocyanate in the polyisocyanate compo-

\* \* \* \* \*